

# UNITED STATES PATENT OFFICE.

THOMAS B. ALLEN, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## PROCESS OF MAKING NITROGENOUS COMPOUNDS.

1,093,819.

Specification of Letters Patent. Patented Apr. 21, 1914.

No Drawing.

Application filed November 9, 1910. Serial No. 591,496.

To all whom it may concern:

Be it known that I, THOMAS B. ALLEN, of Niagara Falls, in the county of Niagara and State of New York, have invented a Process 3 of Making Nitrogenous Compounds, of which the following is a full, clear, and exact description.

My invention has relation to a process of making nitrogenous compounds, which have 10 many valuable properties.

A large number of processes have been described, which have for their object the fixation of atmospheric nitrogen by chemical means. For this purpose it has been proposed to use such substances as titanium, 15 silicon, boron, calcium, and aluminum, using either the elements, or alloys or compounds of these elements.

The process usually consists in passing a 20 current of nitrogen through, or over, the heated element. The nitrogen is formed either by the fractional distillation of liquid air, or, by passing air over heated copper. The nitrogenous compounds prepared in 25 this manner can be used for forming ammonia, and other valuable purposes.

On examination of the elements which readily form nitrogenous compounds, it is seen that they are elements whose carbids 30 are easier to prepare, and cheaper to produce than the elements themselves. This is true of silicon, titanium, calcium, boron, aluminum, and other elements.

I have discovered that nitrogenous compounds 35 can be made, if silicon carbide, and a metal be heated in contact with nitrogen.

I will now describe a method of carrying out my invention using carbide of silicon as the carbide and iron as a suitable metal to 40 react therewith:—I take a mixture of finely divided silicon carbide and iron—for example: a mixture of 85% silicon carbide, and 15% iron, and place this mixture in a suitable furnace, and heat it in contact with 45 nitrogen. A furnace suitable for this operation is a retort having a convenient connection, so that nitrogen can be introduced into the retort as it is absorbed by the reaction.

I heat the mixture to such a temperature 50 that it reacts to form a fritted mass, which state is favorable to the formation of the nitrogenous compounds in using this method. In practice, I have found it preferable to use a temperature of from 1200° to 1800° C. 55 I have also discovered that I may effect the

same result in a slightly different manner, which I will now describe:—I place iron in a suitable vessel, and melt it by any convenient source of heat, and when the iron is in the molten condition, I incorporate silicon 60 carbide in it, and then pass nitrogen through the molten mass. I may also pass a mixture of nitrogen, and silicon carbide through the molten mass of iron. When formed in this manner the nitrogenous product floats to the surface of the bath, and may be tapped off or otherwise removed from the bath. The product obtained is an amorphous grayish material which reacts with alkalis, or other alkaline material to form ammonia. 70

I am not altogether familiar with the chemical nature of the reaction involved in the process, but believe that nitrides, and carbo-nitrides of silicon are formed; and in this specification, and in the following 75 claims, I wish to include these substances under the name of nitrogenous compounds. Substantially the same method is practised when the carbide of some other element than silicon is employed. 80

It will be apparent to those skilled in the art that the described method can be modified in various ways without departing from the spirit and scope of my invention. Thus it can be carried out in any suitable retort or 85 furnace, the nitrogen can be supplied in different ways; other metals than iron may be employed such as copper, nickel, cobalt, chromium and manganese, and various other changes made. 90

I claim:

1. The process of forming nitrogenous compounds which consists in heating silicon carbide, and a metal, with substantially pure nitrogen. 95

2. The process of forming nitrogenous compounds which consists in passing substantially pure nitrogen into contact with a molten metal containing silicon carbide.

3. The process of forming nitrogenous 100 compounds which consists in heating silicon carbide and iron with substantially pure nitrogen.

4. The process of forming nitrogenous compounds, which consists in passing substantially pure nitrogen in contact with molten iron containing silicon carbide. 105

5. The process of forming nitrogenous compounds which consists in causing silicon carbide to react with a metal, and causing 110

substantially pure nitrogen to combine with the reaction-product.

6. The process of forming nitrogeneous compounds, which consists in adding a carbide of an element to iron and dissolving it directly in the molten iron, and passing nitrogen in contact with the molten bath.

7. The process of forming nitrogeneous compounds, which consists in adding a sili-

con carbide to iron and dissolving the silicon carbide directly in the molten iron, and passing nitrogen in contact with the molten bath.

In testimony whereof, I have hereunto set my hand.

THOS. B. ALLEN.

Witnesses:

GEORGE W. CHORMANN,  
L. B. COULTER.